

Dec. 23, 1958

G. FENIAK ET AL  
3-ACYLAMIDO-5-PYRAZOLONE AND 3-ACYLAMIDO-5-ACYLOXPYRAZOLE  
COUPLERS FOR COLOR PHOTOGRAPHY  
Filed Oct. 30, 1956

2,865,748



Fig. 2



GEORGE FENIAK  
ANTHONY LORIA  
WARREN A. RECKHOW  
INVENTORS

BY *Daniel J. Mayne*

*W.H. McNamee*  
ATTORNEY & AGENT

# United States Patent Office

2,865,748

Patented Dec. 23, 1958

1

2,865,748

## 3-ACYLAMIDO-5-PYRAZOLONE AND 3-ACYLAMIDO-5-ACYLOXYPYRAZOLE COUPLERS FOR COLOR PHOTOGRAPHY

George Feniak, Anthony Loria, and Warren A. Reckhow, Rochester, N. Y., assignors to Eastman Kodak Company, Rochester, N. Y., a corporation of New Jersey

Application October 30, 1956, Serial No. 619,151

7 Claims. (Cl. 96—55)

This invention relates to 3-acylamido-5-pyrazolone and 3-acylamido-5-acyloxy-pyrazole couplers for color photography and more particularly to those pyrazolones and pyrazoles having hydroxyalkyl and acyloxyalkyl groups in the 1-position.

3-acylamido-5-pyrazolone couplers for color photography have previously been described and more particularly certain 1-alkyl-3-acylamido-5-pyrazolone couplers. Similarly, certain 5-acyloxy-pyrazole couplers have previously been described. However, the couplers of the present invention are distinct in having the 1-hydroxyalkyl or 1-acyloxyalkyl substituents which confer special properties upon the dyes obtained therefrom in the color development process of color photography. That is, the couplers of the invention yield with the primary aromatic amino silver halide developing agents of color photography magenta dyes which have a somewhat wider range of light absorption than do similar dyes obtained from many of the previously known pyrazolone and pyrazole couplers, which property particularly adapts the new couplers to use with certain benzoylaceto-alkoxyanilide yellow dye-forming couplers in multilayer films for color photography as will be explained in more detail hereinafter.

The pyrazolone and pyrazole couplers of the invention have the following general structures:



and



wherein R represents a member of the class consisting of a hydrogen atom and a carboxylic acid acyl group such as a phenoxyacetyl, heptyl, benzoyl group, etc., R<sub>1</sub> and R<sub>2</sub> each represent a carboxylic acid acyl group such as a phenoxyacetyl, lauroyl, tetracosyl, benzoyl, palmitoyl, heptyl group, etc., and R<sub>3</sub> represents a hydrogen atom, and alkyl group preferably containing from 1 to 4 carbon atoms e. g. methyl, ethyl, n-propyl and n-butyl, or a monocyclic aryl group of the benzene series such as phenyl and nuclear-substituted phenyl.

Representative couplers having these structures are as follows:

- I. 1-(β-hydroxyethyl)-3-[α-(p-palmitamidophenoxy)-acetamido]-5-pyrazolone
- II. 1-[β-(2,4-di-n-amyloxyacetoxymethyl)-3-(2,4-di-n-amyloxyacetamido)-5-(2,4-di-n-amyloxyacetoxymethyl)-pyrazole]
- III. 1-(β-octanoyloxyethyl)-3-(2,4-di-n-amyloxyacetamido)-5-(octanoyloxy)-pyrazole

2

- IV. 1-(β-phenylacetoxymethyl)-3-(2,4-di-n-amyloxyacetamido)-5-(phenylacetoxymethyl)-pyrazole
- V. 1-(β-hydroxyethyl)-3-(2,4-di-n-amyloxyacetamido)-5-pyrazolone
- VI. 1-(β-phenoxyacetoxymethyl)-3-(2,4-di-n-amyloxyacetamido)-5-(phenoxyacetoxymethyl)-pyrazole
- VII. 1-(β-hydroxyethyl)-3-[p-[m-(2,4-di-tert-amyloxyacetamido)benzamido]phenoxyacetamido]-5-pyrazolone
- VIII. 1-[β-(2,4-di-tert-amyloxyacetoxymethyl)-3-(2,4-di-tert-amyloxyacetamido)-5-(2,4-di-tert-amyloxyacetoxymethyl)-pyrazole]
- IX. 1-(β-phenyl-β-hydroxyethyl)-3-(p-nitrophenoxymethyl)-5-pyrazolone
- X. 1-(β-hydroxypropyl)-3-(p-nitrophenoxymethyl)-5-pyrazolone
- XI. 1-(β-hydroxyethyl)-3-[α-(2,4-di-tert-amyloxyacetamido)-5-pyrazolone]
- XII. 1-(β-hydroxyethyl)-3-lauroamido-5-pyrazolone
- XIII. 1-(β-benzoyloxyethyl)-3-benzamido-5-pyrazolone
- XIV. 1-(β-hydroxypropyl)-3-[4-(2,4-di-tert-amyloxyacetamido)phenoxyacetamido]-5-pyrazolone
- XV. 1-(β-hydroxyethyl)-3-tetracosanamido-5-pyrazolone
- XVI. 1-(β-hydroxyethyl)-3-(p-nitrophenoxymethyl)-5-pyrazolone
- XVII. 1-(β-hydroxyethyl)-3-(m-nitrobenzamido)-5-pyrazolone

In the accompanying drawing in Fig. 1 is illustrated by means of spectral absorption curves the preferred utility for the coupler compounds of the invention and the improvement in color reproduction effected by use of the couplers in a particular subtractive color process. In Fig. 2 is shown in greatly enlarged cross-sectional view the appearance of a typical multilayer color film embodying the couplers of the invention.

The benzoylaceto-alkoxyanilide couplers with which the couplers of the present invention are particularly useful are described in the McCrossen et al. U. S. patent application Serial No. 575,099, filed March 30, 1956, and have the following general formula:



wherein R represents an alkyl group of from about 1 to 20 carbon atoms and one of the groups X and Y represents a hydrogen atom and the other represents an organic acid acylamido group.

A particular group of these benzoylaceto-alkoxyanilide couplers efficacious for use with the above couplers of the invention have the above general formula wherein R represents an alkyl group of from about 1 to 20 carbon atoms and one of the groups X and Y represents a hydrogen atom and the other represents the group



wherein R' represents either a hydrogen atom or an alkyl group of from about 1 to 4 carbon atoms.

Representative benzoylaceto-alkoxyanilide couplers having the above formulas are as follows:

- α-[3-[α-(2,4-di-n-amyloxyacetoxymethyl)butyramido]-benzoyl]-2-methoxyacetanilide

## 3

- 3 - benzoylacetamino - 4 - methoxy - (2',4' - di - tert - amylophenoxy)-acetanilide  
 α - {3 - [α - (2,4 - di - tert - amylophenoxy)acetamido]-benzoyl}-2-methoxyacetanilide  
 α - {3 - [α - (2,4 - di - tert - amylophenoxy)butyramido]-benzoyl}-2-methoxyacetanilide  
 α - Benzoyl - 5 - [α - (2,4 - di - tert - amylophenoxy)butyramido]-2-methoxyacetanilide  
 α - {4 - [α - (2,4 - di - tert - amylophenoxy)acetamido]benzoyl}-2-methoxyacetanilide  
 4 - benzoylacetamido - 3 - methoxy - (2',4' - di - tert - amylophenoxy)-acetanilide

The reason why the couplers of the invention are particularly useful with the benzoylacet-o-alkoxyanilide couplers above will be apparent from consideration of the spectral absorption curves shown in the drawing. Curve 1 of Fig. 1 illustrates the region of light absorption of the lemon-yellow dyes obtained in color development of the benzoylacet-o-alkoxyanilide couplers with a particular primary aromatic amino silver halide developing agent.

Curve 2 illustrates the region of absorption of a similar dye made by coupling the same color developing agent with a typical 1-alkyl - 3 - acylamido-5-pyrazolone coupler (1-methyl-3-[4-(2,4-di-tert-amylophenoxyacetamido)-phenoxybutyramido]-5-pyrazolone



Curve 3 illustrates the region of absorption of a similar dye made from the same color developing agent and one of the couplers of the invention (Coupler No. N.II).

Curve 4 illustrates the region of absorption of a dye made from typical known magenta coupler 1-(2,4,6-trichlorophenyl)-3-[3 - (2,4-di-tert-amylophenoxyacetamido)-benzamidol] - 5 - pyrazolone (U. S. 2,600,788) using the same developing agent.

It will be noted from these curves that a rather large gap in absorption appears between curve 1 and curve 4 in the region of wavelength 500 millimicrons which is undesirable because when these dyes are employed together in a subtractive color system, the result is that the yellow colors are reproduced as colors which are more green than desired. Considering curve 2, the absorption maximum is shifted in the right direction but the dye is too sharp-cutting (does not have a wide enough range of absorption). However, when the couplers of the invention (curve 3) are employed with the benzoylacet-o-alkoxyanilide couplers, due to the wider range of light absorption of the dyes obtained from the couplers, the gap in absorption between the yellow and magenta dyes is closed sufficiently resulting in more faithful reproduction of the colors.

The couplers of the invention may be prepared in the following manner:

## COUPLER I

## 1-(β-hydroxyethyl)-3-[α-(p-palmitamidophenoxy)-acetamido]-5-pyrazolone

1-(β-hydroxyethyl) - 3 - (p-nitrophenoxyacetamido)-5-pyrazolone was prepared in the same manner as was 1 - (β-phenyl-β-hydroxyethyl) - 3 - (p-nitrophenoxyacetamido)-5-pyrazolone IX except that 1-(β-hydroxyethyl)-3-amino-5-pyrazolone was used in place of 1-(β-phenyl-β-hydroxyethyl) - 3 - amino-5-pyrazolone. This material was reduced in glacial acetic acid, over 10% palladium on charcoal at ca. 45° C. with hydrogen at a pressure of ca. 30 lbs. per sq. in.. The catalyst was filtered off, the filtrate was concentrated and the residue was treated with 3 equivalents of palmitoyl chloride, in refluxing acetonitrile, in the presence of 3 equivalents of N,N-dimethyl-aniline, for 90 minutes. The triacylated material sepa-

## 4

rated when the reaction mixture was cooled. Twenty g. of this material was treated with 10 ml. of 30% aq. sodium hydroxide in 400 ml. of ethanol. The reaction mixture was warmed to 65° C. for ca. 15 min. The mixture was filtered, the filtrate was acidified with glacial acetic acid and cooled. The solid was recrystallized from a mixture of dimethylformamide/acetonitrile and washed with ether (M. P. 182-184° C.).

| 10 | Anal. | Calc. for C <sub>24</sub> H <sub>46</sub> N <sub>4</sub> O <sub>5</sub> |         | Found |
|----|-------|-------------------------------------------------------------------------|---------|-------|
|    |       | Percent                                                                 | Percent |       |
| C  | 65.6  | 65.2                                                                    |         |       |
| H  | 8.7   | 8.6                                                                     |         |       |
| N  | 10.6  | 10.5                                                                    |         |       |

## COUPLER II

## 1 - [β-(2,4-di-n-amylophenoxyacetoxyl)ethyl]-3-(2,4-di-n-amylophenoxyacetamido) - 5 - (2,4-di-n-amylophenoxyacetoxyl)-pyrazole

A mixture of 2.84 g. of 1-(β-hydroxyethyl)-3-amino-5-pyrazolone, 100 ml. of dry acetonitrile, 18.7 g. of 2,4-di-n-amylophenoxyacetyl chloride and 7.3 g. of N,N-dimethylaniline was stirred and heated to reflux for 3 hours. The mixture was drowned out in water and the product

was recrystallized from ethanol (M. P. 61-63°).

| 35 | Anal. | Calc. for C <sub>65</sub> H <sub>87</sub> N <sub>3</sub> O <sub>8</sub> |         | Found |
|----|-------|-------------------------------------------------------------------------|---------|-------|
|    |       | Percent                                                                 | Percent |       |
| C  | 73.3  | 73.6                                                                    |         |       |
| H  | 9.2   | 9.2                                                                     |         |       |
| N  | 4.3   | 4.6                                                                     |         |       |

## COUPLER III

## 1-(β-octanoyloxyethyl) - 3 - (2,4-di-n-amylophenoxyacetamido)-5-(octanoyloxy)pyrazole

Coupler II was hydrolyzed with two equivalents of sodium hydroxide in aqueous ethanol in the usual manner. The resulting 1-(β-hydroxyethyl)-3-(2,4-di-n-amylophenoxyacetamido)-5-pyrazolone melted at 143-144°. This material was acylated with two equivalents of octanoyl chloride, in the presence of 2 equivalents of N,N-dimethylaniline in dry acetonitrile. The product, after recrystallization from methanol, melted at 50-2° C.

| 55 | Anal. | Calc. for C <sub>25</sub> H <sub>36</sub> N <sub>3</sub> O <sub>4</sub> |         | Found |
|----|-------|-------------------------------------------------------------------------|---------|-------|
|    |       | Percent                                                                 | Percent |       |
| C  | 69.9  | 70.6                                                                    | 70.3    |       |
| H  | 9.5   | 9.9                                                                     |         |       |
| N  | 6.3   | 6.5                                                                     |         |       |

## COUPLER IV

## 1 - (β-phenylacetoxyl)-3-(2,4-di-n-amylophenoxyacetamido)-5-(phenylacetoxyl)pyrazole

65 This compound was prepared in the same manner as was Coupler III except that phenylacetyl chloride was used in place of octanoyl chloride. It melts at 72-3°.

| 70 | Anal. | Calc. for C <sub>39</sub> H <sub>47</sub> N <sub>3</sub> O <sub>6</sub> |         | Found |
|----|-------|-------------------------------------------------------------------------|---------|-------|
|    |       | Percent                                                                 | Percent |       |
| C  | 71.7  | 71.5                                                                    |         |       |
| H  | 7.3   | 7.1                                                                     |         |       |
| N  | 6.5   | 6.3                                                                     |         |       |

5  
COUPLER V1-( $\beta$ -hydroxyethyl)-3-(2,4-di-n-amylphenoxy)acetamido-5-pyrazolone

This compound was prepared in the same manner as was coupler XI below except that 2,4-di-n-amylphenoxyacetyl chloride was used in place of 2,4-di-tert-amylphenoxyacetyl chloride. It melted at 143-144° C.

| Anal. | Calc. for C <sub>23</sub> H <sub>45</sub> N <sub>3</sub> O <sub>4</sub> | Found              |
|-------|-------------------------------------------------------------------------|--------------------|
|       |                                                                         |                    |
| C     | Percent 66.3                                                            | Percent 66.2, 66.6 |
| H     | 8.5                                                                     | 8.5, 8.4           |
| N     | 10.2                                                                    | 10.1               |

## COUPLER VI

1-( $\beta$ -phenoxyacetoxymethyl)-3-(2,4-di-n-amylphenoxyacetamido)-5-(phenoxyacetoxymethyl)pyrazole

This couple was prepared in the same manner as was Coupler IV except that phenoxyacetyl chloride was used as the acylating agent. The product melts at 89.5-91°.

| Anal. | Calc. for C <sub>39</sub> H <sub>47</sub> N <sub>3</sub> O <sub>4</sub> | Found        |
|-------|-------------------------------------------------------------------------|--------------|
|       |                                                                         |              |
| C     | Percent 68.3                                                            | Percent 68.8 |
| H     | 6.9                                                                     | 7.1          |
| N     | 6.1                                                                     | 6.3          |

## COUPLER VII

1-( $\beta$ -hydroxyethyl)-3-{p-[m-(2,4-di-tert-amylphenoxyacetamido)benzamido]phenoxyacetamido}-5-pyrazolone

A mixture of 18.5 g. of 1-( $\beta$ -hydroxyethyl)-3-(p-nitrophenoxyacetamido)-5-pyrazolone (above), 50 ml. of dry acetonitrile, 17.5 g. of benzoyl chloride and 16.6 g. of N,N-dimethylaniline was heated to reflux overnight. The reaction mixture was drowned out in water and the product recrystallized from acetonitrile. Five g. of this material was reduced in tetrahydrofuran, at room temperature, over 10% palladium on charcoal and hydrogen at a pressure of ca. 40 lbs. per sq. in. The catalyst was filtered off and the filtrate was concentrated. The residue was taken up in 50 ml. of dry acetonitrile and treated with 4.1 g. of m-(2,4-di-tert-amylphenoxyacetamido)benzoyl chloride and 1.2 g. of N,N-dimethylaniline. The reaction mixture was refluxed overnight. On cooling, the triacylated compound separated from solution. This was recrystallized from acetonitrile. A mixture of 5 g. of this material, 50 ml. of ethanol, and 8 ml. of 2.5 N aq. sodium hydroxide was refluxed for 30 min., cooled, and acidified with glacial acetic acid. The solid that separated was slurried in boiling acetonitrile and recrystallized from ethanol (M. P. 156-163° C.).

| Anal. | Calc. for C <sub>39</sub> H <sub>47</sub> N <sub>5</sub> O <sub>7</sub> | Found        |
|-------|-------------------------------------------------------------------------|--------------|
|       |                                                                         |              |
| C     | Percent 66.6                                                            | Percent 66.3 |
| H     | 6.9                                                                     | 6.9          |
| N     | 10.2                                                                    | 10.2         |

## COUPLER VIII

1-[ $\beta$ -(2,4-di-tert-amylphenoxyacetoxymethyl)-3-(2,4-di-tert-amylphenoxyacetamido)-5-(2,4-di-tert-amylphenoxyacetoxymethyl)pyrazole

This coupler was prepared in the same manner as was Coupler II except that 2,4-di-tert-amylphenoxyacetyl chloride was used in place of 2,4-di-n-amylphenoxyacetyl chloride. It melted at 113-116°.

## 6

|   | Anal. | Calc. for C <sub>39</sub> H <sub>47</sub> N <sub>3</sub> O <sub>8</sub> | Found        |
|---|-------|-------------------------------------------------------------------------|--------------|
| 5 | C     | Percent 73.3                                                            | Percent 73.1 |
|   | H     | 9.2                                                                     | 8.6          |
|   | N     | 4.3                                                                     | 4.2          |

## COUPLER IX

1-( $\beta$ -phenyl- $\beta$ -hydroxyethyl)-3-(p-nitrophenoxyacetamido)-5-pyrazolone

1-( $\beta$ -phenyl- $\beta$ -hydroxyethyl)-3-amino-5-pyrazolone was prepared by the same method as was used in the preparation of 1-( $\beta$ -hydroxyethyl)-3-amino-5-pyrazolone (below) except that  $\beta$ -phenyl- $\beta$ -hydroxyethylhydrazine (Bull. Soc. Chim. France 6, 71 1939), was used in the place of  $\beta$ -hydroxyethylhydrazine. The 1-( $\beta$ -phenyl- $\beta$ -hydroxyethyl)-3-amino-5-pyrazolone was treated with one equivalent of p-nitrophenoxyacetyl chloride in acetonitrile at room temperature for 90 minutes. The reaction mixture was cooled in ice and filtered. The solid was slurried in water and then in glacial acetic acid. It was recrystallized from n-butanol (M. P. 199-202° C.).

| 25 | Anal. | Calc. for C <sub>19</sub> H <sub>18</sub> N <sub>4</sub> O <sub>6</sub> | Found        |
|----|-------|-------------------------------------------------------------------------|--------------|
|    |       |                                                                         |              |
| 30 | C     | Percent 57.3                                                            | Percent 57.9 |
|    | H     | 4.6                                                                     | 4.9          |
|    | N     | 14.1                                                                    | 14.5         |

## COUPLER X

1-( $\beta$ -hydroxypropyl)-3-(p-nitrophenoxyacetamido)-5-pyrazolone

1-( $\beta$ -hydroxypropyl)-3-amino-5-pyrazolone was prepared by the method used in the preparation of 1-( $\beta$ -hydroxyethyl)-3-amino-5-pyrazolone except that  $\beta$ -hydroxypropylhydrazine (J. Am. Chem. Soc. 76, 1283, 1954), was used in place of  $\beta$ -hydroxyethylhydrazine. The product was acylated with p-nitrophenoxyacetyl chloride by the method used in the acylation of 1-( $\beta$ -hydroxy- $\beta$ -phenylethyl)-3-amino-5-pyrazolone. The product was recrystallized from butanol (M. P. 255-6°).

| 50 | Anal. | Calc. for C <sub>14</sub> H <sub>16</sub> N <sub>4</sub> O <sub>6</sub> | Found        |
|----|-------|-------------------------------------------------------------------------|--------------|
|    |       |                                                                         |              |
| 55 | C     | Percent 50.0                                                            | Percent 50.3 |
|    | H     | 4.8                                                                     | 5.0          |
|    | N     | 16.7                                                                    | 17.0         |

## COUPLER XI

1-( $\beta$ -hydroxyethyl)-3-[ $\alpha$ -(2,4-di-tert-amylphenoxy)acetamido]-5-pyrazolone

1-( $\beta$ -hydroxyethyl)-3-amino-5-pyrazolone, 14.3 g. (0.1 mole),  $\alpha$ -(2,4-di-tert-amylphenoxy)acetyl chloride, 93 g. (0.3 mole), and dimethylaniline, 36.3 g. (0.3 mole), were heated in 500 ml. of dry acetonitrile at reflux overnight. The next morning the reaction mixture containing the triacylated pyrazolone was poured into 2.5 l. of cold water and the oil that separated was washed several times with water by decantation.

The oil layer was then taken up in 500 ml. of 3A alcohol containing 16.8 g. of potassium hydroxide and allowed to stand two hours at room temperature. The mixture was acidified by the addition of 20 ml. of acetic acid contained in 80 ml. of water, and the solid which precipitated was filtered, washed well with water, and air dried.

The product was crystallized from toluene twice, getting white needles melting between 105-106° C.

| Anal. | Calc. for C <sub>33</sub> H <sub>45</sub> N <sub>3</sub> O <sub>5</sub> (401) | Found   |
|-------|-------------------------------------------------------------------------------|---------|
|       | Percent                                                                       | Percent |
| C     | 66.5                                                                          | 66.5    |
| H     | 8.7                                                                           | 8.6     |
| N     | 10.5                                                                          | 10.2    |

1-( $\beta$ -hydroxyethyl)-3-amino-5-pyrazolone

$\beta$ -hydroxyethylhydrazine, 71 g. of 70% material, and ethyl- $\beta$ -ethoxy- $\beta$  iminopropionate, 112 g. were mixed and 1 ml. of acetic acid was added as a catalyst. The mixture was stirred vigorously and cooled so that the temperature would not rise above 50° C. After about one hour no more heat was evolved and a solid precipitated out of the solution. The solid was filtered, washed well with cold water, and crystallized from ethyl alcohol. White, thin plates, melting between 160-162° C., were obtained which gave the following chemical analysis:

| Anal. | Calc. for C <sub>6</sub> H <sub>9</sub> N <sub>3</sub> O <sub>2</sub> (143) | Found   |
|-------|-----------------------------------------------------------------------------|---------|
|       | Percent                                                                     | Percent |
| C     | 42.0                                                                        | 42.3    |
| H     | 6.3                                                                         | 6.6     |
| N     | 29.4                                                                        | 29.7    |

## COUPLER XII

1-( $\beta$ -hydroxyethyl)-3-lauramide-5-pyrazolone

This compound was prepared in the same manner as was 1-( $\beta$ -hydroxyethyl)-3-[ $\alpha$ -(2,4-di-tert-amylphenoxy)-acetamido]-5-pyrazolone XI except that lauroyl chloride was used as the acid chloride. It was recrystallized from ethyl alcohol and melted at 112-115° C.

| Anal. | Calc. for C <sub>21</sub> H <sub>35</sub> N <sub>3</sub> O <sub>3</sub> | Found   |
|-------|-------------------------------------------------------------------------|---------|
|       | Percent                                                                 | Percent |
| C     | 66.0                                                                    | 66.2    |
| H     | 10.2                                                                    | 10.4    |
| N     | 11.0                                                                    | 10.8    |

## COUPLER XIII

1-( $\beta$ -benzoyloxyethyl)-benzamido-5-pyrazolone

A mixture of 7.2 g. of 1-( $\beta$ -hydroxyethyl)-3-amino-5-pyrazolone, 150 ml. of dry acetonitrile, 22.5 g. of benzoyl chloride and 18 g. of N,N-dimethylaniline was refluxed for 4 hours and left to stand overnight. A soln. of 20 ml. of 30% aq. NaOH in 50 ml. of water was added and the mixture was stirred for 2½ hours. Water (250 ml.) was added, and the mixture was acidified with glacial acetic acid. The solid was filtered off and recrystallized from ethyl alcohol (M. P. 204-205° C.).

| Anal. | Calc. for C <sub>19</sub> H <sub>17</sub> N <sub>3</sub> O <sub>4</sub> | Found   |
|-------|-------------------------------------------------------------------------|---------|
|       | Percent                                                                 | Percent |
| C     | 65.4                                                                    | 65.1    |
| H     | 5.1                                                                     | 4.8     |
| N     | 12.5                                                                    | 12.0    |

## COUPLER XIV

This compound is prepared from Coupler X by reduction of the nitro group and reaction with 2,4-di-tert-amylphenoxyacetyl chloride.

## COUPLER XV

1-( $\beta$ -hydroxyethyl)-3-tetracosanamido-5-pyrazolone

This compound was prepared by the same method used for preparing 1-( $\beta$ -hydroxyethyl)-3-[ $\alpha$ -(2,4-di-tert-amylphenoxy)acetamido]-5-pyrazolone XI. It too was

crystallized from toluene and had a melting point between 167-169° C.

| Anal. | Calc. for C <sub>29</sub> H <sub>55</sub> N <sub>3</sub> O <sub>5</sub> (493) | Found   |
|-------|-------------------------------------------------------------------------------|---------|
|       | Percent                                                                       | Percent |
| C     | 70.6                                                                          | 70.5    |
| H     | 11.1                                                                          | 11.4    |
| N     | 8.5                                                                           | 8.4     |

The coupler compounds of the invention find usage in a wide variety of photographic color processes wherein silver halide emulsions are developed in the presence of the couplers. For example, Couplers Nos. IX, X, XIII, XVI, XVII, XVIII are most useful in color developing solutions for the development of multilayer color films in which some or all of the emulsion layers are devoid of coupler compounds. A typical color developing solution in which such couplers can be incorporated is as follows:

|                                       |     |
|---------------------------------------|-----|
| 2-amino-5-diethylaminotoluene sulfate | 2.5 |
| Sodium sulfite (anhydrous)            | 5   |
| Sodium carbonate (anhydrous)          | 20  |
| Potassium bromide                     | 2   |
| Water to 1000 cc.                     |     |

The couplers can be incorporated into the developer compositions by first dissolving them in a solvent such as isopropyl alcohol and adding this solution to an alkaline developer composition. About 3 grams of the couplers of the invention are suitable for use in developer compositions such as the above.

Color developing solutions thus containing the couplers of the invention are used in well known subtractive color processes. A color film containing at least one emulsion layer and preferably two or three emulsion layers sensitized to different regions of the spectrum is exposed to a subject, developed in a black-and-white developer followed by selective reversal exposure and the exposed emulsion layer color developed with the above developing solution containing one of the coupler compounds appropriate for the particular emulsion layer which has been reversal exposed.

The other couplers which are substantially nondiffusing in emulsion layers such as gelatino silver halide emulsion layers are most appropriate for use in silver halide emulsion layers designed for color processes of the well known negative-positive and reversal types. These less diffusible couplers, for example, Couplers Nos. I-VIII and XI-XV can be dispersed in an emulsion layer such as a gelatino silver halide emulsion layer by means of coupler solvents including cellulose esters, natural and synthetic resins and organic crystalloidal materials having a boiling point above about 170° C., as described in the Mannes et al. U. S. Patent 2,304,940, granted December 15, 1942, and the Jelley et al. U. S. Patent 2,322,027, granted June 15, 1943. The optimum quantity of coupler to use in the emulsion layer (as in the case of 40 use in a color developer) can be determined by simple experiment and will depend somewhat upon the coupling activity of the particular coupler, the silver halide content of the emulsion layer, the particular process in which the emulsion is to be used and other factors well known in the art of emulsion making.

A typical procedure for making an emulsion and color film therefrom is as follows:

Six-tenths gram of 1-[ $\beta$ -(2,4-di-n-*amylphenoxyacetox*)-ethyl]-3-(2,4-di-n-*amylphenoxyacetamido*)-5-(2,4-di-n-*amylphenoxyacetox*)-pyrazole (Coupler II) was dissolved in 1.2 g. of tricresylphosphate by heating to 120° C. with stirring. This solution was mixed with 17.7 ml. of 10% gelatin solution containing 2 ml. of 5% Alkanol B. The mixture was passed through a colloid mill four times to disperse the coupler solution.

Fourteen ml. of water used to rinse out the colloid mill was added to the dispersion, which was then made up to a total of 40 g. with additional water. This dispersion was mixed at 40° C. with 8.5 ml. of a melted sensitive silver bromoiodide emulsion of the type described by Trivelli and Smith in the Phot. Jour. Vol. 79, pp. 330-31, (1939), and the mixture was coated on a cellulose acetate support. After drying, the coating was exposed under an image and developed in a 2-amino-5-diethylaminotoluene developing composition to form a 10 silver and magenta dye negative image. The silver image and residual silver halide were removed with ferricyanide-hypo bleach leaving a negative image having maximum absorption at a wavelength of 528 m $\mu$ .

The couplers of the invention can be employed in a 15 multilayer color film in conjunction with the benzoylacet-o-alkoxyanilide couplers for the purposes mentioned as follows: A multilayer film was prepared using emulsion melts made in a manner similar to that described in the single layer example above: (1) a gelatin dispersion of 20 a cyan coupler, 1-hydroxy-2-[ $\delta$ (2,4-di-tert-*amyl*phenoxy)-*n*-butyl]-naphthamide dissolved in tricresylphosphate was added to a red-sensitive gelatin silver-halide emulsion and coated as the bottom layer, (2) a gelatin dispersion of a magenta coupler, 1-[ $\beta$ -(2,4-di-*n*-amylphenoxyacetoxo) - ethyl] - 3 - (2,4 - di - *n* - amylphenoxyacetamido) - 5 - (2,4 - di - *n* - amylphenoxyacetoxo) - parazole (Coupler II), dissolved in tricresyl phosphate was added to a green-sensitive gelatin silver-halide emulsion and coated as the middle layer, and (3) a gelatin dispersion of a yellow coupler,  $\alpha$ -{3-[ $\alpha$ -(2,4-di-tert-*amyl*phenoxy)acetamido]benzoyl} - 2 - methoxyacetanilide dissolved in di-*n*-butylphthalate, was added to an unsensitized gelatin silver-halide emulsion and coated as the 25 top sensitive layer over a Carey Lea silver yellow filter interlayer. The film was exposed and processed as in the same manner as the single layer material above.

A multilayer color film prepared as just described is illustrated in Fig. 2 in the drawings wherein layer 20 represents a support such as a cellulose ester film base, layer 21 represents a red-sensitive silver halide emulsion layer containing a cyan coupler, layer 22 represents a green-sensitive silver halide emulsion layer containing the coupler compound of the invention, layer 23 represents a yellow filter layer such as a Carey-Lea silver 40 filter layer and layer 24 represents a blue-sensitive silver halide emulsion layer containing the mentioned benzoylacet-o-alkoxyanilide coupler. Such a film can be developed directly to a color negative or indirectly to a color positive by well known reversal methods.

The 3-acylamido-5-acyloxyprazole couplers of the invention can be used in emulsion or color developing solutions in substantially the same manner as described for the 5-pyrazolone couplers of the invention above. These prazole couplers are particularly useful in that they have lower melting points and higher solubility in coupler solvents than the corresponding 5-pyrazolones, although the 5-pyrazole compounds tend to be somewhat less active couplers. It will be noted from the syntheses of, for example, Couplers VII and XI that the mono-55 acylated couplers are readily obtained by hydrolysis of the triacylated 5-pyrazoles disclosed, the 3-acylamido group of the acylated 5-pyrazoles being more resistant to hydrolysis.

The color developing agents used for development of 65 emulsion layers in the presence of the novel coupler compounds include the well known primary aromatic amino silver halide developing agents such as the phenylenediamines including the alkyl phenylenediamines and alkyl toluene diamines as well as the p-aminophenols in which the amino group is unsubstituted. The N-alkyl sulfonamido alkyl-p-phenylenediamine developing agents of U. S. Patent 2,193,015 are particularly useful for the development of emulsion layers in the presence of the couplers of the invention.

The silver halide component of the emulsion layers is not especially critical and may be, for example, silver bromoiodide, silver bromide or silver chloride, etc., depending upon the results desired. Likewise, the emulsions which are developed in the presence of the novel couplers may consist of single-layer or differentially sensitized multilayer films.

The hydrophilic colloid vehicle of the emulsions may be selected from known types including gelatin, hydrolyzed cellulose esters, polyvinyl alcohol and other natural and synthetic organic colloids.

The examples and compounds set forth in the present specification are illustrative only and it is to be understood that our invention is to be taken as limited only by the scope of the appended claims.

What we claim is:

1. A photographic silver halide emulsion containing a coupler compound of the class consisting of those having the general formulas



and



wherein R represents a member of the class consisting of a hydrogen atom and a carboxylic acid group, R<sub>1</sub> and R<sub>2</sub> each represent a carboxylic acid acyl group and R<sub>3</sub> represents a member of the class consisting of a hydrogen atom, an alkyl group of from 1 to 4 carbon atoms and a monocyclic aryl group of the benzene series.

2. A photographic silver halide emulsion containing a coupler compound having the general formula



wherein R represents a carboxylic acid acyl group.

3. A photographic silver halide emulsion containing a compound of the class consisting of 1-[ $\beta$ -(2,4-di-*n*-amylphenoxy - acetoxy)ethyl] - 3 - (2,4 - di - *n* - amylphenoxyacetamido) - 5 - (2,4 - di - *n* - amyl - phenoxyacetoxo) - pyrazole, 1 - ( $\beta$  - phenylacetoxethyl) - 3 - (2,4 - di - *n* - amylphenoxyacetamido) - 5 - (phenylacetoxo) - pyrazole, 1 - ( $\beta$  - phenoxyacetoxethyl) - 3 - (2,4 - di - *n* - amylphenoxyacetamido) - 5 - (phenoxyacetoxo) - pyrazole, 1 - ( $\beta$  - hydroxyethyl) - 3 - [ $\alpha$ -(2,4 - di - tert - *amyl*phenoxy)acetamido] - 5 - pyrazolone, 1 - ( $\beta$  - hydroxyethyl) - 3 - (p - nitrophenoxoacetamido)-5-pyrazolone.

4. A multilayer color film comprising a support having thereon a silver halide emulsion designated in claim 1 sensitive to green light and a silver halide emulsion sensitive to blue light containing a coupler compound having the general formula



wherein R represents an alkyl group of from 1 to 20 carbon atoms and one of the groups X and Y represents a hydrogen atom and the other represents an organic acid acylamido group.

5. A multilayer color film comprising a support having thereon a silver halide emulsion designated in claim 1 sensitive to green light and a silver halide emulsion sensi-

11

sensitive to blue light containing a coupler compound having the general formula



wherein R represents an alkyl group of from 1 to 20 carbon atoms and one of the groups X and Y represents a hydrogen atom and the other represents the group



wherein R' represents a member of the class consisting of a hydrogen atom and an alkyl group of from 1 to 4 carbon atoms.

6. A multilayer color film comprising a support having thereon a silver halide emulsion designated in claim 1 and sensitive to green light, and a silver halide emulsion sensitive to blue light containing a coupler compound of the class consisting of

- $\alpha$  - {3 - [ $\alpha$  - (2,4 - di - n - amylphenoxy)butyramido] - benzoyl}-2-methoxyacetanilide
- 3 - benzoylacetamino - 4 - methoxy - (2',4' - di - tert - amylphenoxy)-acetanilide
- $\alpha$ -{3 - [ $\alpha$  - (2,4-di-tert-amylphenoxy)acetamido]-benzoyl}-2-methoxyacetanilide
- $\alpha$  - {3 - [ $\alpha$  - (2,4 - di - t - amylphenoxy)butyramido] - benzoyl}-2-methoxyacetanilide
- $\alpha$  - Benzoyl - 5 - [ $\alpha$  - (2,4 - di - tert - amylphenoxy)butyramido]-2-methoxyacetanilide

5

$\alpha$  - {4 - [ $\alpha$  - (2,4 - di - tert - amylphenoxy)acetamido] - benzoyl}-2-methoxyacetanilide

4 - benzoylacetamido - 3 - methoxy - (2',4' - di - tert - amylphenoxy)-acetanilide

10

7. A method of producing a colored photographic image in a developable silver halide emulsion layer which comprises developing said layer with a primary aromatic amino silver halide developer in the presence of a coupler compound of the class consisting of those having the general formulas



and



wherein R represents a member of the class consisting of a hydrogen atom and a carboxylic acid acyl group, R<sub>1</sub> and R<sub>2</sub> each represent a carboxylic acid acyl group and R<sub>3</sub> represents a member of the class consisting of a hydrogen atom, an alkyl group of from 1 to 4 carbon atoms and a monocyclic aryl group of the benzene series.

20

References Cited in the file of this patent

UNITED STATES PATENTS

- |           |              |               |
|-----------|--------------|---------------|
| 2,721,798 | Loria et al. | Oct. 25, 1955 |
| 2,772,161 | Loria et al. | Nov. 27, 1956 |

UNITED STATES PATENT OFFICE  
CERTIFICATE OF CORRECTION

Patent No. 2,865,748

December 23, 1958

George Feniak et al.

It is hereby certified that error appears in the printed specification of the above numbered patent requiring correction and that the said Letters Patent should read as corrected below.

Column 3, line 35, for "NII" read -- XII --; column 10, line 33, after "acid" insert -- acyl --.

Signed and sealed this 5th day of May 1959.

(SEAL)

Attest:

KARL H. AXLINE

Attesting Officer

ROBERT C. WATSON  
Commissioner of Patents